

## UNITED STATES PATENT OFFICE

PAUL LOGUE, OF BIRMINGHAM, ALABAMA, AND THEODORE W. SCHILB, OF ST. LOUIS, MISSOURI, ASSIGNORS TO SWANN RESEARCH, INC., A CORPORATION OF ALABAMA

## POLISHING COMPOSITION AND METHOD OF PREPARING SAME

No Drawing.

Application filed June 3, 1931. Serial No. 541,950.

This invention relates to polishing bases and in particular to a dicalcium phosphate polishing base.

The object of this invention is to produce a dry polishing base composed of hydrated or partially dehydrated dicalcium phosphate dihydrate. Another object is to produce a dicalcium phosphate polishing base of low abrading power.

Hitherto it has been extremely difficult to produce a polishing base of uniform finely divided particles sufficiently soft so that surfaces which were polished therewith would not be excessively abraded. At the same time it was desirable that the particles of the polishing base be of sufficient hardness so that a polishing effect could be obtained without the expenditure of too much effort. We have now discovered that a polishing base comprising partially dehydrated dicalcium phosphate dihydrate which has been prepared according to the method herein described has a very low abrading power combined with sufficient hardness so that a good polish may be obtained.

Measurement of the abrading power of polishing agents consists merely in comparing the weight of material removed from a reference substance by means of various polishing agents applied under controlled conditions. Experiments which we have made to compare the abrading power of the herein described partially dehydrated dicalcium phosphate dihydrate with anhydrous dicalcium phosphate have shown that the former has only 1/10 to 1/30 of the abrading power of the latter.

The material herein described may be used as a metal polish or for lacquered or plated surfaces, especially on automobiles, as a jeweler's polish or as a dentifrice base.

We have discovered that by controlling the conditions under which dicalcium phosphate is formed we are enabled to produce a dry, hydrated or partially dehydrated dicalcium phosphate dihydrate of low abrading power suitable for use as or for introduction into polishing compositions. We have further discovered that by the addition of aluminum phosphate or aluminum hydrate into the

reaction mixture in which precipitated dicalcium phosphate is being formed, the production of the dry dicalcium phosphate in a hydrated or partially dehydrated form with a low degree of abrading power is rendered extremely simple.

The addition of aluminum hydrate into the reacting mass causes the formation of phosphate of aluminum, hence we may add this aluminum compound directly into the reacting mixture or may form it by reaction of the hydrate and phosphoric acid.

Our new product may be used in the dry state as a polishing agent or it is preferably combined with other ingredients which assist in polishing or cleaning.

For cleaning metals the dry, partly hydrated dicalcium phosphate may be moistened with orthodichlor-benzene, naphtha or benzene. To use as a jeweler's polish, the dry powder is mixed with an alcohol, preferably ethyl alcohol or acetone, and applied as a paste. Mixed with water to form a paste, it can be used directly as a tooth paste. It is particularly valuable because of its low abrading power as an ingredient of polishes for lacquered surfaces for which purpose it is mixed with sufficient water to form a paste to which a small amount of soap may be added if desired.

The following examples illustrate our method of preparing a polishing base composed of hydrated or only partly dehydrated dicalcium phosphate of low polishing power.

## Example I

Add sufficient lime slurry of 9-11° Bé. strength to a water solution of phosphoric acid of between 9 and 11° Bé. so that substantially all of the acid is neutralized and dicalcium phosphate formed. During the reaction the temperature should be kept below 45° C. The precipitate of dicalcium phosphate hydrate may be separated from the mother liquor by filtration and the wet filter cake will contain approximately 30% excess moisture. The filter cake is now dried at a temperature of 80° C. The drying operation is preferably carried out in a vacuum

55

60

65

70

75

80

85

90

95

100

with stirring until a sample of the product shows an ignition loss of 14-21 per cent of moisture. When this degree of drying has been obtained, the product is ground to a fine 5 powder and is suitable for incorporation into a polish in the usual manner.

*Example II*

Add sufficient lime to phosphoric acid to 10 form dicalcium phosphate as in the previous example. In addition, add a sufficient quantity of aluminum phosphate so that the dried product will contain approximately 3% of aluminum phosphate. Aluminum hydrate 15 may be used in place of aluminum phosphate, in which case sufficient additional phosphoric acid is employed to precipitate the phosphate of aluminum. During the reaction of the lime and phosphoric acid, the temperature is maintained below 45° C. in order 20 to assure the formation of the hydrated dicalcium phosphate. After reaction the slurry containing the precipitated dicalcium phosphate and aluminum phosphate is filtered. 25 The cake is now dried, in this case however, because of the protecting action of the aluminum phosphate in the cake, the temperature may be increased to 104° C. without any danger of forming the anhydrous dicalcium 30 phosphate. Drying, which may or may not be carried out in a vacuum, and is preferably done with stirring, is continued until the product shows an ignition loss of between 14 and 21 per cent.

35 Some variations may be made in the amount of aluminum phosphate or hydrate added; however, it is desirable to keep the content of aluminum phosphate between 1 and 3 per cent if a higher drying temperature 40 than 80° C. is employed. As pointed out above, when 3 per cent of aluminum phosphate is present in the product, a maximum temperature of 104° C. is permissible during drying; when less than this amount is 45 present the temperature of drying is decreased so that a product having a low abrading power is obtained. The maximum temperature permissible during drying of the dicalcium phosphate in the absence of any 50 aluminum phosphate is in the neighborhood of 80° C.

The ignition loss of the product is preferably maintained between 14 and 21 per cent 55 by weight. It is determined by heating a two-gram sample at a temperature of 800° C. for 30 minutes or until constant weight is obtained.

A dried product made in the above manner 60 and having an ignition loss of substantially less than 21% will comprise partially dehydrated dicalcium phosphate dihydrate. The abrading power of this product, however, will not be appreciably higher because of the 65 presence of this partially dehydrated dical-

cium phosphate, if the procedure given above is carefully followed.

While we have described our invention in but two forms, it will be obvious to those skilled in the art that it is not so limited, but 70 is susceptible of various other changes and modifications, without departing from the spirit thereof, and we desire, therefore, that only such limitations shall be placed thereupon as are imposed by the prior art or 75 as are specifically set forth in the appended claims.

What we claim is:

1. A polishing base comprising dicalcium phosphate dihydrate which has been partially 80 dehydrated and a relatively small amount of aluminum phosphate.

2. A polishing base comprising dicalcium phosphate dihydrate which has been partially dehydrated and containing from 1 to 3 per 85 cent of aluminum phosphate.

3. A polishing base composed of dicalcium phosphate dihydrate having a low abrading power and which has been dehydrated until it has an ignition loss of between 14 and 21 90 per cent, and sufficient aluminum phosphate to raise the drying temperature of the product slightly above normal temperature.

In testimony whereof we affix our signatures.

PAUL LOGUE.  
THEODORE W. SCHILB.

100

105

110

115

120

125

130